

1

3,761,262

PHOTOGRAPHIC COLOR DEVELOPING PROCESS  
Karl-Wilhelm Schranz, Opladen, and Erwin Schön and  
Wolfgang Hünicken, Leverkusen, Germany, assignors  
to Agfa-Gevaert Aktiengesellschaft, Leverkusen, Ger-  
many

No Drawing. Filed Aug. 18, 1971, Ser. No. 172,891  
Claims priority, application Germany, Aug. 20, 1970,  
P 20 41 325.6

Int. Cl. G03c 5/00, 5/38, 5/44  
U.S. Cl. 96—22 6 Claims

### ABSTRACT OF THE DISCLOSURE

The formation of color fog during the bleaching step 15 of color processing, particularly rapid color processing, is suppressed by including certain sulphydrazides in the bleach bath, and preferably further adding a large quantity of thiosulfate as well as a color coupler that couples with developer oxidation products without forming a dye. 20

This invention relates to a photographic color developing process, more particularly a rapid-processing technique, using aromatic sulphydrazides as agents to prevent 25 the formation of fog upon bleaching.

It is known to produce color-photographic images by color-forming development of exposed silver halide emulsion layers in the presence of suitable color couplers capable of reaction with the oxidation product of the 30 color-forming developer substance, to form a dye image. Aromatic compounds containing primary amino groups, especially those of the p-phenylene diamine type, are normally used as color-forming developers. After color development, the photographic material has to be treated 35 with a bleaching bath and a fixing bath, or with a bleach-fixing bath, in order to remove image silver and any silver halide still present after development. The bleaching substances used are oxidizing agents which not only oxidize the image silver but also some residual color developers that are still present in the photographic emulsion after the development operation. This oxidation, in the presence of color couplers, leads to undesired formation of a dye-fog of azomethine or indoquinone dye, referred to below as bleach fog.

To avoid this defect in processing, it is known to rinse the developed material rising rinsing times that are long in relation to the total processing time after development, or alternatively the material has to be pretreated with a stopping, or stopping and fixing bath, before the bleaching or bleach-fixing operation. Both these measures are obstacles to quick processing in the true sense and involve additional costs. Another method is to carry out the bleaching or bleach-fixing operation in the presence of special substances which inhibit formation of bleach fog. Examples of compounds that have been recommended for this purpose include N-hydroxymorpholine, N-amino morpholine, certain 3-pyrazolidone derivatives and certain amino-phenol derivatives; unfortunately, these compounds are relatively unstable in the bleaching or bleach-fixing bath, or if they are sufficiently stable, they are not sufficiently active.

It is among the objects of the present invention to provide improved anti-foggants for the bleaching bath to prevent formation of the bleach fog.

We have now found a photographic process for making color-photographic images including color development of an image-wise-exposed color photographic material comprising at least one silver halide emulsion layer, bleaching and fixing or bleach-fixing, wherein bleaching or bleach-fixing is performed in the presence of an aro-

2

matic sulphydrazide corresponding to the following formula



in which R<sup>1</sup> represents hydrogen, nitro or carboxyl, and R<sup>2</sup> represents hydrogen, halogen such as chlorine or bromine, or alkyl or alkoxy having up to three carbon atoms, preferably methyl or methoxy.

The following are examples of suitable aromatic sulphydrazides which prevent bleach fog:



55 The aforementioned substances are added to the bleaching or bleach-fixing bath in quantities of preferably from 0.5 to 10 g. per litre. It is also possible to briefly treat the developed material with an aqueous solution of the compound according to the invention before bleaching. In this instance, it is advisable to employ a relatively high concentration of the sulphydrazides in the pretreatment bath. Useful results are obtained for example with aqueous pretreatment baths containing from 5 to 50 g. per litre of the sulphydrazides.

65 The compounds used according to the invention can of course also be used in the conventional processing of color photographic materials, in which case intermediate rinsing is usually carried out between the developer bath, the bleaching bath and fixing bath, or the bleach-fixing bath. However, they can be used with particular advantage in so-called "rapid-processing," which is preferably carried out at slightly elevated temperatures and in which

